

## UNITED STATES PATENT OFFICE

2,549,137

METHOD FOR REMOVAL OF OXIDES OF  
COPPER FROM SURFACES OF ALLOYS  
OF COPPER AND SILVERArchy F. Slover, Los Angeles, Calif., assignor to  
Kelite Products, Inc., Los Angeles, Calif., a cor-  
poration of CaliforniaNo Drawing. Application March 10, 1947,  
Serial No. 733,727

2 Claims. (Cl. 134—41)

1

This invention relates to a method of treating silver alloyed with copper for the purpose of removing copper oxides from the surface thereof.

Silver is alloyed with copper for the purpose of hardening silver. Thus, for example, sterling silver consists of an alloy of 92½% silver and of 7½% copper. For hardening sterling silver, it is annealed by heating to about 1400° F., followed by quenching in cold water. This annealing process results in the formation of cuprous and cupric oxides on the surface of the metal. Previous to the present invention, it has been necessary to treat the metal with acids, such as sulphuric and nitric acid to remove these copper oxide coatings. These treatments with sulphuric and nitric acid to remove these copper oxide coatings result in a considerable loss in silver.

It is the object of the present invention to provide a process by means of which silver alloys with copper may be treated for the removal from the surface thereof of copper oxides without the treating solution dissolving any of the silver of the alloy.

I have discovered that these copper oxides may be satisfactorily removed by treating the metal with hot solutions of acid reacting aluminum salts. Thus, for example, a dilute aqueous solution of any aluminum salt having an acid reaction when hot, such, for example, as aluminum sulphate, aluminum chloride or aluminum ammonium sulphate will successfully remove copper oxides from silver alloys, without dissolving substantially any of the silver.

While any of the acid solutions of aluminum salts which are soluble in water may, when

2

heated, operate satisfactorily, I prefer to employ solutions of aluminum sulphate. The amount of aluminum sulphate in solution is not critical and a suitable value is three ounces of aluminum sulphate per gallon of water.

The treatment is conducted hot, preferably boiling the solution while in contact with the metal. A suitable treating time for treating, for example, sterling silver, is an annealing process of from three to ten minutes.

This invention is of the scope set forth in the appended claims.

I claim:

1. A process of treating alloys of silver and copper for the removal of copper oxides, which process consists in treating the alloy with a hot solution of an acid reacting aluminum salt of a strong inorganic acid.
2. A process of treating silver alloyed with copper for removal of copper oxides from the surface thereof, which process consists in treating the alloy with a hot solution of an acid-reacting aluminum salt of a strong inorganic acid essentially consisting of aluminum sulphate.

ARCHY F. SLOVER.

## REFERENCES CITED

The following references are of record in the file of this patent:

## UNITED STATES PATENTS

| Number    | Name      | Date           |
|-----------|-----------|----------------|
| 542,382   | Toobe     | July 9, 1895   |
| 1,278,744 | Poetschke | Sept. 10, 1918 |